

July 27, 1937.

P. KNOCHE

2,088,523

MULTICOLOR PHOTOGRAPHIC MATERIAL

Filed Feb. 8, 1935

Fig. 1

Light sensitive layer  
including a dyestuff



Light insensitive layer containing  
undeveloped silver or colloidal silver

Fig. 2

Light sensitive layer including a  
dyestuff forming substance



Light insensitive layer containing  
a substance which prevents the  
formation of dyestuff

Paul Knoche

INVENTOR

BY

F. Gerald Toye

ATTORNEY

## UNITED STATES PATENT OFFICE

2,088,523

## MULTICOLOR PHOTOGRAPHIC MATERIAL

Paul Knoche, Berlin, Germany, assignor to Bela Gaspar

Application February 8, 1935, Serial No. 5,665  
In Germany February 14, 1934

7 Claims. (Cl. 95-8)

In the production of multi-color photographs having a plurality of colored layers poured one on to the other a creeping of the dyestuffs into adjacent layers frequently has a very disturbing effect, in which connection remedy is sought to be obtained by precipitation of the dyestuffs in the layers.

Despite these precautions there is frequently encountered the disadvantage that the dyestuff in the lowermost layer diffuses into the backing or support and colors the latter. This veil of color cannot be removed by the usual means without variation of the image situated above the same, as the means employed for destroying the dyestuff in the actual photographic or image bearing layers are unable to react with the backing or support.

Now it has been found that the small percentage of dyestuff which creeps or diffuses into the backing or support, intermediate or anti-halation layers or in fact any non-image bearing layers at all which remain uncolored in the finished image may be readily removed by incorporating therein substances which destroy the dyestuff diffusely only in these layers, either in themselves or in conjunction with the subsequent baths to which the image is subjected. The reference to dyestuffs is also intended to include dyestuff-forming substances. In this case, in addition to the dyestuff-destroying agents, there may also be included chemical substances which prevent the formation of the dyestuff or act as a chemical resist.

There are a variety of ways in which the invention may be carried into effect. The dyestuff-destroying agents are incorporated in direct fashion in the backing or support. If indifferent dyestuff-destroying agents are employed, that is to say—substances which, whilst destroying the dyestuff at the desired points, will have no adverse effect on the image during the normal time of treatment thereof, there is added to the backing or support or other layer which is to remain ultimately uncolored either a small quantity of colloidal silver or an exposed silver halide emulsion. In the first case the metallic silver will undergo the same reactions as the silver in the sensitized image bearing layer or layers and destroy the dyestuff diffusely, the silver also being contained diffusely in the particular layer. If on the other hand exposed silver halide is employed, this requires to pass through the developing and fixing baths in order to form metallic silver. Oxidizing or coupled reactions are also

suitable for the process according to the invention.

It is also possible to incorporate in the backing or support or intermediate or other layer the same substances as included in the sensitized image bearing layer. The process according to the invention is particularly suitable for paper or films having a plurality of differently colored layers, in which the substances according to the invention are incorporated in the backing or support.

In the accompanying drawing Fig. 1 and Fig. 2 represent sections of film.

Referring to these figures layer *a* represents a light sensitive layer which may contain a dyestuff or a dyestuff forming substance. Layer *b* represents a light insensitive layer containing a substance which prevents the formation of a dyestuff.

The light sensitive layer *b* may be the backing or support for layer *a* or it may be any other non-image bearing layer. It is to be understood that in the following examples wherein reference is made to the backing or support as the layer treated with a substance preventing the formation of a dyestuff, that such expression includes any other non-image bearing layer into which it is desired to prevent diffusion.

## Examples

1. There is added to the backing or support, which usually consists of hardened gelatine, a certain proportion of colloidal silver.

2. To the backing or support of a film or paper there is added a small amount of exposed silver halide gelatin.

In the developer this silver halide gelatin will be developed and form in the backing or support a sufficient quantity of metallic silver. In the subsequent baths to which the image is subjected this metallic silver will undergo the same reactions as the silver in the developed image. In the destruction of the dyestuff, for example with an acid thiocarbamide solution, the backing or support containing diffusely the metallic silver will destroy diffusely any dyestuff which has crept into the same.

3. There is added to the backing or support an insoluble oxidizing agent, such as zinc chromate. In this case the destruction of the dyestuff will take place by oxidation.

4. The sensitized layers contain leuco esters, i. e., dyestuff-forming substances, which are converted into dyestuff by oxidation. There is then incorporated in the backing or support a reduc-

30

35

40

45

50

55

ing agent, such as mercurous chloride, which will oppose the formation of the dyestuff.

- 5 The small amount of silver which is contained in the backing or support, intermediate or other layer will have no interfering effect in the observation of the image. If, as frequently the case, the final bath employed is a silver solvent, all traces of silver in the backing or support will disappear entirely.
- 10 Beyond the additions referred to it is also possible to make use of many others assuming they do not affect the sensitiveness and transparency of the sensitized layers. They should, therefore, also not creep from the backing or support, intermediate or other layer into the upper layers.
- 15 What I claim as new and desire to secure by Letters Patent is:

- 20 1. A photographic material comprising colored light sensitive layers and an uncolored light insensitive layer adjacent thereto, said uncolored layer containing a proportion of exposed silver halide, said proportion of silver halide when passed through a developing bath, yielding a quantity of metallic silver sufficient to assist in the destruction of any dyestuff diffusing into said uncolored layer so as to prevent the formation of a color veil therein.
- 25 2. A photographic material comprising a light sensitive photographic layer containing a substance for coloring an image, and a light insensitive layer adjacent thereto containing an insoluble chemical substance which reacts to destroy a compound necessary to the formation of a color veil in said light insensitive layer.
- 30 3. A photographic material comprising a light sensitive photographic layer containing a dyestuff forming substance convertible into a dyestuff by oxidation, and a light insensitive layer adjacent thereto containing a reducing agent for preventing oxidation of any dyestuff forming substance diffusing into said light insensitive

layer to prevent the formation of a color veil in said light insensitive layer.

4. A photographic material comprising a light sensitive photographic layer containing a dyestuff, and a light insensitive layer adjacent thereto containing a chemical substance which reacts with a developing bath to produce an agent which assists in the destruction of any dyestuff diffusing into said light insensitive layer from said light sensitive layer to prevent the formation of a permanent color veil in said light insensitive layer.

5 5. A photographic material comprising a light sensitive silver halide emulsion layer containing a dyestuff adapted to be reacted with a silver image formed in said layer to destroy the dyestuff where silver is present, and a light insensitive layer adjacent said light sensitive layer containing a proportion of exposed silver halide adapted to be converted into metallic silver upon development to assist in the destruction of any dyestuff diffusing into said light insensitive layer, whereby the formation of a color veil in said light insensitive layer is prevented.

6. A photographic material comprising a light sensitive silver halide emulsion layer containing a dyestuff adapted to be reacted with a silver image formed in said layer to destroy the dyestuff where silver is present, and a light insensitive layer adjacent thereto containing a proportion of colloidal silver for assisting in the destruction of any dyestuff diffusing into said light insensitive layer to prevent the formation of a color veil in said light insensitive layer.

7. A photographic material comprising a support, and applied to said support a light sensitive photographic layer containing a substance for coloring an image, said support having incorporated therein an insoluble chemical substance which reacts to destroy a compound necessary to the formation of a color veil in said support.

PAUL KNOCHÉ.